# EUROPEAN PATENT SPECIFICATION

(11) **EP 2 209 649 B1**
(45) Date of publication and mention of the grant of the patent: **25.07.2012**
(21) Application number: 08844473.2
(22) Date of filing: 31.10.2008
(51) Int. Cl.: B41M 7/00, B41M 3/14, B41M 5/50, B41M 5/52, D21H 19/66, G03G 21/04

(54) **COPY PROTECTED PAPER**
KOPIERGESCHÜTZTES PAPIER
PAPIER PROTÉGÉ CONTRE LA COPIE

(30) Priority: 31.10.2007 EP 07119762
(43) Date of publication of application: 28.07.2010
(73) Proprietor: Nederlandse Organisatie voor Toegepast -Natuurwetenschappelijk Onderzoek TNO, 2628 VK Delft (NL)
(72) Inventor: HOVENS, Irene Antoinette Petra, NL-5913 CD Venlo (NL); BATENBURG, Lawrence Fabian, NL-5652 EJ Eindhoven (NL); TIMMERMANS, Johannes Wilhelmus, NL-6714 GG Ede (NL); RENTROP, Cornelis Hermanus Arnoldus, NL-5616 AE Eindhoven (NL); JETTEN, Jan Matthijs, NL-3701 JL Zeist (NL); TURKENBURG, Daniël Hendrik, NL-5643 DM Eindhoven (NL)
(74) Representative: Hatzmann, Martin
(86) International application number: PCT/NL2008/050683
(87) International publication number: WO 2009/058013

(56) References cited:
- WO-A-03/012733
- JP-A- 4 095 989
- JP-A- 2004 188 950
- DATABASE WPI Week 198745 Thomson Scientific, London, GB; AN 1987-318783 XP002476593 & JP 62 049199 B (OIKE KOGYO KK) 17 October 1987 (1987-10-17)

## Description

The invention is directed to copy protected paper, to a method for producing said paper, and the use of a specific layer for copy protection of paper.

Paper is used as a medium for recording all kinds of printed information. Normally such information can be copied, for instance by means of a photocopier. However, in particular when the information contained on the paper is valuable (such as in the case of banknotes, cheques, licences, certificates, paper with copyright information, or other security paper) it is not desirable that the original can easily be copied.

In the prior art several attempts have been made to protect a paper original from being copied. Some of these attempts are directed at adjusting photocopiers, others are directed at using special inks or toners, still others are directed at the use of specific printing technologies. It would, however, be desirable to have a paper that is protected against making copies. Ideally, the copy of such a paper would be unreadable or unrecognisable. However, it would already be advantageous to be able to immediately distinguish the copy from the original.

JP-A-2004 188 950 describes a paper having a black camouflage pattern printed thereon. A layer of fluorescent ink is provided on top of the black camouflage pattern. Information printed on this paper can be read by irradiating the paper with black light and the fluorescent layer emits coloured light. A copy of the original turns out black because of the black camouflage pattern. Major disadvantages of this paper are that the original paper has a black colour and that the information on the original can only be read by irradiating the paper with black light.

JP-A-4 201562 describes a paper on which is provided a resin layer containing transparent fine particles having reflective ability and reflective pigment. Incident light transmits through the transparent fine particles and is reflected by the reflective pigment, which is emitted from the transparent fine particles. Due to the reflective pigment, the resin layer is visible. Furthermore, in order to have the desired effect, a combination of transparent fine particles with the reflective pigment is required.

JP-A-04 095 989 describes a copy-protected paper that comprises an absorption layer that absorbs light and a reflection layer between the absorption layer and the surface of the paper. The reflection layer comprises transparent layers having refraction indexes different from each other.

EP-A-0 171252 describes a transparent sheet, which sheet contains an authenticating retroreflective image. The sheet comprises a monolayer of transparent microlenses, preferably glass microspheres having average diameters in the range of 10 to 300 µm. The sheet is applied as an overlay on top of an already printed original document.

Object of the invention is to at least partially overcome the disadvantages of the prior art.

Another object of the invention is to protect a paper from being copied using a layer that is not visible.

A further object of the invention is to provide a paper that is protected from copying in that the copy can be immediately distinguished from the original.

Another object of the invention is to provide an accessible and cheap method for protecting printable paper from being copied.

The inventors found that one or more of these objects can be met by providing a paper with specific refractive index properties.

Accordingly, in a first aspect the invention is directed to a copy protected paper comprising a printable paper having, on a side to be printed or a printed side, a first transparent layer, wherein said first transparent layer has a difference in refractive index with
i) said paper; or
ii) an optional second transparent layer being provided on said paper on the side to be printed or the printed side,
wherein said difference in refractive index is at least 0.05, and wherein the first transparent layer further comprises 1-50wt.% of inorganic particles having an average particle size of 0.5-200 nm.

The term "copy protected paper" as used herein refers to a paper that can contain printed information and of which the copied information is at least significantly different than the original information. Thus, when the original information contained on the copy protected paper is copied, the information on the copy is at least significantly different than the original information. The copied information can for instance be in the form of a photocopy, but also a scan of the original, for instance by a digital scanner, is considered a copy in the context of this invention.

The copy protected paper of the invention thus comprises a printable paper which is overlaid with at least one transparent layer. If desirable, the transparent layer can be printed on. The paper can be printed on before application of the layer. Of course, also the combination of these possibilities (i.e. a paper which is printed on before application of the transparent layer and which is to be printed thereafter) is an option.

The transparent layer of the copy protected paper of the invention can also be a multilayer, comprising more than one layer, such as 2-20 layers. It is preferred that such a multilayer design has at least one time a refractive index difference of 0.0.5 between different layers, preferably at least 2 times, more preferably at least 3 times, and even more preferably at least 5 times. In a more preferred embodiment the multilayer design has at least one time a refractive index difference of 0.1 between different layers. The one or more transparent layers can suitably be prepared by wet coating techniques and/or by gas phase deposition.

The difference in refractive index between the transparent layer and the paper or the optional second transparent layer causes the paper to be copy protected. Information that is optionally printed on the paper under the transparent layer and/or that is printed on top of the transparent layer, is visible under low angles, typically angles of less than 90°, preferably less than 70°, more preferably 70°-50°. However, under substantially right angles, typically angles of 30°-90°, preferably angles of 70°-90°, more preferably angles of 90°, the information becomes invisible because of total reflection.

In the most extreme form the transparent layer under substantially right angles functions as a mirror-and totally reflects the light of a copying device. As almost all copying devices shine light onto the original under right angles or substantially right angles, the paper is protected from being copied by almost all copying devices.

The difference in refractive index is at least 0.05, preferably at least 0.1. The refractive index can reliably be measured by refractometry. The refractive index is usually measured or expressed in index at 550 nm. In a more preferred embodiment the difference in refractive index is at least 0.2, preferably at least 0.5, more preferably 0.5-1.0. The larger the difference in refractive index, the wider the angle under which incident light is totally reflected. At very big differences in refractive index, such as differences of more than 1.0, a large extent of light is reflected so that information on the original becomes hard to distinguish with bare eye. For instance, if the information is in the form of a text, the original may be hard or impossible to read.

In principle, the refractive index of the transparent layer can be either lower or higher than the refractive index of the paper or optional second transparent layer. In practice, it has been found convenient to prepare a transparent layer with a refractive index that is higher than the refractive index of the paper or optional second transparent layer.

The term "paper" as used in this application is meant to refer to all types of cellulose-based products in sheet or web form. Examples of suitable papers include bank paper, drawing paper, printer paper (such as inkjet paper), copier paper and photographic paper. Cellulose-based paper normally has a refractive index of about 1.56 (Dissertation of Tapio Fabritius, Acta Univ. Oul., C 269, April 2007, Finland, ISBN 978-951-42-8404-5).

In accordance with the invention it is also possible that the paper is coated. Coating may exist of an inorganic coating such as china clay, TiO₂ and/or latex. Also resin coated paper can be used.

The one or more transparent layers can suitably independently from each other comprise an organic polymer as a binder. In a preferred embodiment the organic polymer is selected from the group consisting of starch, cellulose, polyvinylalcohol and derivatives thereof. Particularly, preferred organic polymers are for instance copolymers of polyvinyl alcohol and polyvinyl acetate optionally with itaconic acid, carboxymethylcellulose, and amylase free potato starch (for instance the amylopectin potato starch Eliane™, commercially obtainable from AVEBE).

The one or more transparent layers of the paper according to the invention can independently from each other comprise inorganic particles. If particles are present, these particles should have an average particle size, which is smaller than the wavelength of light in the visible in order to prevent scattering of light, which would make the layer non-transparent. Thus, the particles can have an average particle size of 0.5-200 nm, preferably 0.6-100 nm, more preferably 0.7-50 nm, as determined by transmission electron microscopy. The first transparent layer comprises 1-50 wt% of inorganic particles having an average particle size of 0.5-200 nm. It is preferred that the particles are present as non-agglomerated, or at least hardly agglomerated, individual particles. Thus, in a preferred embodiment the above-mentioned average particle sizes refer to the average particle sizes of individual particles. In principle, the particles can have any shave. However, it is preferred that the particles are non-spherical.

The inorganic particles can suitably have a refractive index of at least 0.4, preferably at least 1.0, more preferably 1.0-4.0, and most preferably 2.0-4.0 as determined by refractometry.

Inorganic particles can for instance be selected from the group consisting of TiO₂ (refractive index of the particles about 2.2), SnO₂, Si (refractive index of the particles about 4.0), Ag (refractive index of the particles about 1.35), Au (refractive index of the particles about 0.47), C(diamond) (refractive index of the particles about 2.4), ZnO (refractive index of the particles about 2.0), ZrO₂ (refractive index of the particles about 2.2), CeO₂ (refractive index of the particles about 2.3), Hf₂O₃ (refractive index of the particles about 1.9), mica particles (refractive index of the particles about 1.50 to 1.70) and (organically modified) clays (refractive index of the particles about 1.50). Commercial mica particles may be coated with rutile (TiO₂ structure with refractive index of about 2.63), tin oxide (refractive index of about 2), and/or various iron oxides.

It was found that if the transparent layer closest to the paper comprises mica, preferably mica coated with rutile titanium dioxide, tin oxide, and/or iron oxide, the copy protection is enhanced. Without wishing to be bound by theory, it is believed that this is due to additional reflection of the incoming light by the underlying mica layer.

In a preferred embodiment, the first transparent layer comprises inorganic particles having a refractive index difference of at least 0.2 compared to the paper or the optional second transparent layer, preferably a difference of at least 1.0, more preferably at least 1.5 as determined by refractometry. It was found that inorganic particles with a refractive index that strongly differs from the refractive index of the paper or the optional second transparent layer significantly contribute to the copy protection of the paper.

The inorganic particles can be dispersed in the organic polymer binder. Preferably, the particles are dispersed homogeneously and the formation of aggregates is prevented. Aggregate formation could lead to an aggregate particle size which is larger than the wavelength of light, thereby causing light scattering and in turn leading to a non-transparent layer. In order to increase the compatibility of the particles with the organic polymer it is possible to modify the surface of the inorganic particles. Typically, the surface of the inorganic particles is modified with organic compounds comprising ammonium, phosphonium, carboxylic, siloxane, and/or hydroxylic groups.

Another possibility to make the inorganic particles more compatible with the organic polymer binder is to add one or more surfactants to the transparent layer. Suitable surfactants include block-copolymers. Suitable blocks for use in the block-copolymers for instance include polyethylene oxide, maleic acid anhydride, carbonic acid, alcohol, and polyethylene glycol, polypropylene, polyethylene, polystyrene, polymethylmethaclylate, polyamide, and polyethylene oxide. The block-copolymers may be provided with a functional terminus, such as a carbonic acid group, a hydroxyl group, or an epoxy group. It is also possible to combine the addition of surfactants with a surface modification of the inorganic particles.

The amount of the particles in the one or more transparent layers can be chosen in a wide range. It is preferred that the one or more transparent layers independently from each other comprise 1-50 wt.%, preferably 20-40-wt.%, more preferably 30-40 wt.% of the inorganic particles, with the provision that the first transparent layer comprises 1-50 wt.% of inorganic particles having an average particle size of 0.5-200 nm. The ratio between the inorganic particles and the organic polymer in the transparent layer is preferably at least 5:95, more preferably at least 50:50. When the ratio between inorganic particles and organic polymer binder in the transparent layer is more than 60:60, this can cause problems in the preparation of the layer. Accordingly, the ratio between the inorganic particles and the polymer binder in the transparent layer is preferably in the range of 2:98-40:60, more preferably 10:90-20:80. A high amount of inorganic particles compared to the amount of organic polymer may cause problems in viscosity of a coating solution that can be used to prepare the transparent layer. In addition, such a high relative amount of inorganic particles can lead to less transparent layers, If the amount of inorganic particles is very low it becomes more difficult to realise a sufficiently high difference in refractive index with the paper.

In a special embodiment of the invention, the inorganic particles are quantum dots (semiconductor nanop articles), which are optionally fluorescent.

The one or more transparent layer may further independently from each other comprise one or more dyes. The dyes can be inorganic, organic, or a mixture of inorganic and organic dyes can be used. Suitable organic dyes are for instance acridine dyes, anthraquinone dyes, diarylmethane dyes, triarylmethane dyes, azo dyes, phtalocyanine dyes, diazonium dyes, quinone dyes, azin dyes, indamine dyes, indophenol dyes, oxazin dyes, oxazone dyes, thiazin dyes, thiazole dyes, xanthene dyes, fluorene dyes, rhodamine dyes, and fluorone dyes. The inventors found that the provision of a dye in the first transparent layer can cause an additional show-through effect during copying of the original, *i.e.* when information is provided on both sides of the original, the single-sided copy contains the information of both sides of the original.

It was found that the presence of one or more dyes in the first transparent layer can lead to a show-through effect. Without wishing to be bound by theory, it is believed that this show-through effect relates to a spectral overlap of the absorption of the dye in the transparent layer with the emission spectrum of the lamp of the photocopying machine or scanner. It is believed that the show-through effect increases when this spectral overlap is increased.

Therefore it in a preferred embodiment, the first transparent layer comprises a dye which has an absorption spectrum that overlaps with the emission spectrum of the lamp of the photocopier.

If one or more dyes are included, it is preferred that the dyes are strongly absorbing. The dye can have for example a molar extinction coefficient at its absorption maximum of at least 10 000 Lmol⁻¹cm⁻¹, preferably at least 20 000 Lmol⁻¹cm⁻¹, more preferably at least 50 000 Lmol⁻¹cm⁻¹. In practice there are only few dyes with a molar extinction coefficient of more than 200 000 Lmol⁻¹cm⁻¹.

In a special embodiment, the one or more transparent layers independently from each other comprise one or more emitting dyes, preferably fluorescent dyes. Suitable fluorescent dyes include fluoresceins, rhodamines, coumarins, and the like. Also phosphorescent dyes can be used. Irradiation by a lamp of a photocopying machine can bring the emitting dye in an excited state after which the dye can emit light, either by fluorescence or by phosphorescence. This emitted light can interfere with the photocopying process. Fluorescent dyes are preferred over phosphorescent dyes, because fluorescence is a faster relaxation process than phosphorescence.

When the one or more transparent layers comprise emitting dyes, it is preferred that the copy protected paper is provided with means to concentrate the emitted light. Such means can for instance be grooves or pits in one or more transparent layers. Such grooves or pits in should have a dimension larger than the wavelength of the emitted light. It was found that such grooves or pits can efficiently concentrate the emitted light, thereby increasing the interference with the photocopying process. The grooves or pits, which are hardly visible in the original because of their small size (typically smaller than 100 µm, preferably smaller than 50 µm), appear in the copy as bright areas as a result of the interfering emitted light.

For very thin layers the observed total reflection effect becomes small. In such cases a copy of the information printed on the copy protected paper may not be not unrecognisable, but still distinguishable from the original. Preferably, the one or more single transparent layers on the paper preferably have a layer thickness of at most 1 000 nm, preferably at most 500 nm, more preferably at most 200 nm. The layer thickness can be reliably measured by a profilometer. It is in general difficult to fabricate single layers with a layer thickness of more than 5 µm. In a preferred embodiment, the one or more single transparent layers have a layer thickness of 100-500 nm for the wet chemically applied layers. Single layers applied by gas phase deposition are to be applied at a thickness of 50 to 150 nm. For better performance the layers can be stacked. Suitably a stack can comprise at least 2 layers, preferably at least 5 layers, more preferably at least 15 layers.

In a further aspect the invention is directed to a method of preparing a copy protected paper as described above, comprising
- providing a printable paper, wherein said paper is optionally printed on thereby providing said paper with a printed side;
- optionally providing said paper with a transparent layer on the side to be printed or on the printed side;
- providing a coating composition, optionally comprising an organic polymer, which coating composition, when dried, has a refractive index that differs at least 0.05, preferably at least 0.1, from the refractive index of said printable paper or from the refractive index of said transparent layer;
- applying said coating composition onto the printed side or to a side of said paper to be printed on; and
- drying acid coating composition,

The optional transparent layer can be applied before or after applying the coating composition onto the paper to provide a transparent coating that comprises 1-50 wt.% of inorganic particles having an average particle size of 0.5-200 nm.

The coating solution can simply be prepared by mixing the components together in a suitable mixing process. Optionally, solvents can be added. Suitable solvent for instance include water, alcohols (such as ethanol, pronanol, isopropanol, butanol, and the like), ketones (such as aceton, methylethylketone, and the like). Subsequently, the coating composition is applied to the optionally printed paper. This can be performed by any coating method known in the art, such as air knife coasting, immersion (dip) coating, gap coating, curtain coating, rotary screen coating, revere roll coating, gravure coating, metering rod (meyer bar) coating, slot die (extrusion) coating, or hot melt coating. At least the side to be printed should be coated in accordance with the method of the invention. It is possible to coat more than one side of the paper,

As mentioned above the paper can be a coated paper. Optionally, the coated paper can be printed on, and subsequently the optionally printed paper can be overlaid with the transparent layer.

In yet a further aspect the invention is directed to a method of preparing a copy protected paper as describe above, comprising
- providing a printable paper, wherein said paper is optionally printed on thereby providing said paper with a printed side;
- optionally providing said paper with a transparent layer on the side to be printed or on the printed side;
- applying a transparent layer that comprises 1-50wt.% of inorganic particles having an average particle size of 0.5-200nm onto the printed side or to a side of said paper to be printed on by a gas phase deposition process, wherein said layer, after being applied by gas phase deposition, has a refractive index that differs at least 0.05, preferably at least 0.1, from the refractive index of said printable paper or from the refractive index of said optional transparent layer.

The optional transparent layer can be applied before or after application of the transparent layer that is applied by gas phase deposition. In a preferred embodiment, multiple transparent layers are deposited by gas phase deposition. It is preferred that such a multilayer design has at least one time a refractive index difference of 0.05 between different layers, preferably at least 2 times, more preferably at least 3 times, and even more preferably at least 5 times. In a more preferred embodiment, the multilayer design has at least one time a refractive index difference of 0.1 between different layers.

The gas phase deposition process can suitably be chosen from chemical vapour deposition, plasma enhanced chemical vapour deposition, atmospheric pressure chemical vapour deposition, sputter deposition, electron beam physical vapour deposition, or the life. Furthermore, various materials may be used for the gas phase deposited layers. The layers can be deposited from metal organic precursors, such as tetraethoxy ortho silicate (TEOS), tetraisopropoxytitanate, tin chloride, metals like Al, Au, Cr, Cu, Ge, Hf, In, Sn, Ir, Mo, Nb, Ni, Pt, Ta, Ti, W, Zr or Zn, or their oxides. Also combinations of these materials are possible.

The porosity of the layer can assist in creating a high refractive index coating. Layers with lower porosity in general have a higher refractive index difference with the paper. Therefore, it is preferred that the porosity of the first transparent layer is less than 10 % as measured by ellipsometry, preferably less than 1 %, more preferably less than 0.1 %.

Also disclosed is a method of protecting a printed paper or a paper to be printed from being copied comprising applying on the paper, on the printed side or on the side to be printed, at least a first transparent layer as defined above.

In yet a further aspect the invention is directed to the use of the first transparent layer as defined herein above as a copy-protection for information printed or to be printed on a paper.

The copy protected paper of the invention can e.g. be used for copy sensitive information, such as the information on paper money, banknotes, cheques, licences, certificates, vouchers, tickets, papers with copyright information., or any other security paper.

### Examples

### Preparation of coasting solutions

### TEOS (coating solution 1 (25 % wlw))

10.86 g TEOS (tetraethoxysilane) and 22.84 g IPA (isopropylalcohol) was mixed at 0 °C (ice bath) for 15 minutes while adding dropwise 4.4 g 1M HNO₃ and 1.7 g of demineralised water. Next this solution was refluxed at 80 °C for 2 hours. This solution is mentioned as the stock solution 1 (25 % w/w). The refractive index of this coating is 1.45.

### PVA mica sparkle solution

A 7% (w/w) solution of polyvinyl alcohol (Mowiol^{®} 18-88, Mw 130k Da Fluka, refractive index of 1.50) in DEMI water is prepared. Mica (Sparkle 139P, Exterior Mearlin^{®}) is added up to a concentration of 10 % (w/w). This type of mica based particles is coated with TiO₂ and tin oxide.

### PVA mica magna pearl solution

A 7 % (w/w) solution of polyvinyl alcohol (Mowiol^{®} 18-88, Mw 130k Da Fluka, refractive index of 1.50) in DEMI water is prepared. Mica (Magna Pearl^{®} 5000) is added up to a concentration of 10 % (w/w). Magna Pearl^{®} 4000 can also be used instead of Magna Pearl^{®} 5000.

### Dipping procedure

The papers were dipped in the coating solutions attached to a glass plate to prevent wrinkling. The papers were totally submerged for 25 seconds before the dipping process (upward motion) was started.

### Examp de 1- TEOS (25 % w/w)

Regular copying paper (79 g/m²), having a refractive index or 1.56, was coated with the coating solution 1. The coating was dipped in the stock solution 1 with an upward velocity of 1 maws leaving behind 15.4 g/m² of coating. The difference in refractive index between the copying paper and the dried coating was 0.11. Figure 1 shows the results copied on a Xerox^{®} standard copier (black and white). Figure 1A is a digital photo of the original coated paper, Figure 1B is a result of a copied coated paper at high sensitivity.

### Standard CVD coating procedure

Alternating layers of hafniumdioxide and silicon dioxide were applied at specific layer thicknesses. The standard CVD layer contains 11 layers as specified below:
1, hafnium dioxide: 71.28 nm refractive index 1.95
2, silicon dioxide: 94.50 nm refractive index 1.46
3, hafnium dioxide: 71.28 nm refractive index 1.95
4, silicon dioxide: 94.50 nm refractive index 1.46
5, hafnium dioxide: 71.28 nm refractive index 1.95
6, silicon dioxide: 94.50 nm refractive index 1.46
7, hafnium dioxide: 53.50 nm refractive index 1.95
8, silicon dioxide: 94.50 nm refractive index 1.46
9, hafnium dioxide: 53.50 nm refractive index 1.95
10, silicon dioxide: 94.50 nm refractive index 1.46
11, hafnium dioxide: 53.50 nm refractive index 1.95
Hence, the CVD coating resulted in a multilayer with a difference in retroactive index of 0.49 between each layer.

### Example 2 - Coating composition 1

First regular photopaper (233.5 g/m²) was printed with text. After that a standard PVA mica magna pearl^{®} layer was applied using a doctor blade of 60 µm which was left to dry after which a standard CVD layer as described above was applied. On these layers additional text can be written with a pencil. Figure 2A shows a photograph of a layer of composition 1 on paper viewed under 90 degrees. Figure 2B is a photograph of the same layer viewed under a small angle. Figure 2C shows copies of the layer as depicted in A and B at varying intensity settings of a copy machine.

### Example 3 - Coating composition 2

First regular photopaper (233.5 g/m²) was printed with text. After that a standard PVA mica sparkle layer was applied using a doctor blade of 60 µm which was left to dry after which a standard CVD layer as described above was applied. Figure 3A shows a photograph of a layer of composition 2 on paper viewed under 90 degrees. Figure 3B is a photograph of the same layer viewed under a small angle. Figure 3C shows copies of the layer as depicted in A and B at varying intensity settings of a copy machine. On these layers additional text can bewas written with a pencil (see Figure 4; 4A: photograph of a layer of composition 2 on paper viewed under 90 degrees; 54: photograph of the same layer viewed under a small angle; 54: copies of the layer as depicted in A and B at varying intensity settings of a copy machine).

## Claims

1. Copy protected paper comprising a printable paper having, on a side to be printed or a printed side, a first transparent layer, wherein said first transparent layer has a difference in refractive index with
i) said paper; or
ii) an optional second transparent layer being provided on said paper on the side to be printed or the printed side,
wherein said difference in refractive index is at least 0.05, and
wherein the first transparent layer further comprises 1-50 wt.% of inorganic particles having an average particle size of 0.5-200 nm.

2. Copy protected paper according to claim 1, wherein the first transparent layer comprises an organic polymer, preferably the organic polymer is selected from the group consisting of starch, cellulose, polyvinylalcohol, and derivatives thereof.

3. Copy protected paper according to any one of the preceding claims, wherein the first transparent layer further comprises inorganic particles having an average particle size of 0.6-100 nm, preferably 0.7-50 nm, and wherein preferably said particles are non-spherical.

4. Copy protected paper according to claim 3, wherein said non-spherical particles are in the form of platelets having a width to height aspect ratio of 10 or more, wherein the orientation of the particles is such that the average angle between the plane of the platelets and the plane of the paper is less than 60°, preferably less than 45°, more preferably less than 20°.

5. Copy protected paper according to any one of the preceding claims, wherein said difference in refractive index is at least 0.1, preferably at least 0.2, more preferably at least 0.5, and even more preferably 0.5-1.5.

6. Copy protected paper according to any one of the preceding claims, wherein the inorganic particles are selected from the group consisting of TiO₂, SnO₂, Si, Ag, Au, C(diamond), ZnO, ZrO₂, CeO₂, Hf₂O₃, optionally coated mica, and optionally organically modified clay.

7. Copy protected paper according to any one of the preceding claims, wherein the first transparent layer comprises 20-40 wt.%, preferably 30-40 wt.% of inorganic particles.

8. Copy protected paper according to any one of the previous claims, wherein the total thickness of the sum of transparent layers is at most 1 000 nm, preferably at most 500 nm, and more preferably at most 200 nm.

9. Copy protected paper according to any one of the preceding claims, comprising at least 2 transparent layers, preferably 2-20 transparent layers, more preferably the transparent layer closest to the paper comprises mica, preferably mica coated with rutile titanium dioxide, tin oxide, and/or iron oxide.

10. Copy protected paper according to any one of the preceding claims, wherein the inorganic particles have a refractive index of at least 0.4, preferably at least 1.0, more preferably 1.0-4.0, and most preferably 2.0-4.0 as determined by a refractometer.

11. Copy protected paper according to any one of the preceding claims, wherein the surface of the inorganic particles is modified with one or more organic compounds, preferably said one or more organic compounds comprise ammonium, phosphonium, carboxylic, siloxane, and/or hydroxylic groups.

12. Copy protected paper according to any one of the previous claims, wherein said first transparent layer comprises one or more dyes, preferably said dye is an organic dye selected from the group consisting of acridine dyes, anthraquinone dyes, diarylmethane dyes, triarylmethane dyes, azo dyes, phtalocyanine dyes, diazonium dyes, quinone dyes, azin dyes, indamine dyes, indophenol dyes, oxazin dyes, oxazone dyes, thiazin dyes, thiazole dyes, xanthene dyes, fluorene dyes, rhodamine dyes, and fluorone dyes, and/or wherein said dye is an emitting dye.

13. Copy protected paper according to any one of the previous claims, wherein the paper is chosen from the group consisting of bank paper, drawing paper, printer paper, inkjet paper, copier paper and photographic paper.

14. Method of preparing a copy protected paper according to any one of claims 1-13, comprising
- providing a printable paper, wherein said paper is optionally printed on thereby providing said paper with a printed side;
- optionally providing said paper with a transparent layer on the side to be printed or on the printed side;
a)
- providing a coating composition, optionally comprising an organic polymer, which coating composition, when dried, has a refractive index that differs at least 0.05, preferably at least 0.1, from the refractive index of said printable paper or from the refractive index of said transparent layer;
- applying said coating composition onto the printed side or to a side of said paper to be printed on; and
- drying said coating composition to provide a transparent coating that comprises 1-50 wt.% of inorganic particles having an average particle size of 0.5-200 nm, or
b)
- applying a transparent layer that comprises 1-50 wt.% of inorganic particles having an average particle size of 0.5-200 nm onto the printed side or to a side of said paper to be printed on by a gas phase deposition process, wherein said layer, after being applied by gas phase deposition, has a refractive index that differs at least 0.05, preferably at least 0.1, from the refractive index of said printable paper or from the refractive index of said optional transparent layer.

15. Use of a transparent layer as defined in any one of claims 1-12 as a copy protection for information printed or to be printed on a paper.

## Patentansprüche

1. Kopiergeschütztes Papier, umfassend ein bedruckbares Papier mit, auf einer zu bedruckenden Seite oder einer bedruckten Seite, eine erste transparente Schicht, wobei die erste transparente Schicht einen Unterschied im Brechungsindex aufweist mit
i) dem Papier; oder
ii) einer optionalen zweiten transparenten Schicht, bereitgestellt auf dem Papier auf der zu bedruckenden Seite oder der bedruckten Seite,
wobei der Unterschied im Brechungsindex mindestens 0,05 ist, und
wobei die erste transparente Schicht ferner 1-50 Gewichtsprozent anorganischer Partikel mit einer durchschnittlichen Partikelgröße von 0,5-200 nm aufweist.

2. Kopiergeschütztes Papier nach Anspruch 1, wobei die erste transparente Schicht ein organisches Polymer umfasst, vorzugsweise ein organisches Polymer ausgewählt aus der Gruppe bestehend aus Stärke, Zellulose, Polyvinylalkohol und Derivaten davon.

3. Kopiergeschütztes Papier nach einem der vorhergehenden Ansprüche, wobei die erste transparente Schicht ferner anorganische Partikel mit einer durchschnittlichen Partikelgröße 0,6-100 nm, vorzugsweise 0,7-50 nm umfasst, und wobei vorzugsweise die Partikel nicht kugelförmig sind.

4. Kopiergeschütztes Papier nach Anspruch 3, wobei die nicht kugelförmigen Partikel die Form von Plättchen mit einem Seitenverhältnis Breite zu Höhe von 10 oder mehr haben, wobei die Orientierung der Partikel so ist, dass der durchschnittliche Winkel zwischen der Ebene der Plättchen und der Ebene des Papiers kleiner als 60°, vorzugsweise kleiner als 45° und noch bevorzugter kleiner als 20° ist.

5. Kopiergeschütztes Papier nach einem der vorhergehenden Ansprüche, wobei der Unterschied im Brechungsindex mindestens 0,1, vorzugsweise mindestens 0,2, bevorzugter mindestens 0,5 und noch bevorzugter 0,5-1,5 ist.

6. Kopiergeschütztes Papier nach einem der vorhergehenden Ansprüche, wobei die anorganischen Partikel ausgewählt sind aus der Gruppe bestehend aus TiO₂, SnO₂, Si, Ag, Au, C(Diamant), ZnO, ZrO₂, CeO₂, Hf₂O₃, optional beschichtetem Glimmer und optional organisch modifiziertem Ton.

7. Kopiergeschütztes Papier nach einem der vorhergehenden Ansprüche, wobei die erste transparente Schicht 20-40 Gewichtprozent, vorzugsweise 30-40 Gewichtprozent anorganische Partikel umfasst.

8. Kopiergeschütztes Papier nach einem der vorhergehenden Ansprüche, wobei die Gesamtdicke der Summe der transparenten Schichten höchstens 1 000 mm, bevorzugt höchstens 500 nm und noch bevorzugter höchstens 200 nm ist.

9. Kopiergeschütztes Papier nach einem der vorhergehenden Ansprüche, umfassend mindestens 2 transparente Schichten, vorzugsweise 2-20 transparente Schichten, bevorzugter die transparente Schicht, die dem Papier am nächsten ist, Glimmer umfasst, vorzugsweise Glimmer, beschichtet mit Rutil-Titandioxid, Zinnoxid und/oder Eisenoxid.

10. Kopiergeschütztes Papier nach einem der vorhergehenden Ansprüche, wobei die anorganischen Partikel einen Brechungsindex von mindestens 0,4, vorzugsweise mindestens 1,0, bevorzugter 1,0-4,0 und am bevorzugtesten 2,0-4,0 haben, wie ermittelt durch ein Refraktometer.

11. Kopiergeschütztes Papier nach einem der vorhergehenden Ansprüche, wobei die Oberfläche der anorganischen Partikel mit einer oder mehreren organischen Verbindungen modifiziert ist, wobei die eine oder mehreren organischen Verbindungen vorzugsweise Ammonium, Phosphonium, Carbonsäure, Siloxan und/oder Hydroxylsäure umfassen.

12. Kopiergeschütztes Papier nach einem der vorhergehenden Ansprüche, wobei die erste transparente Schicht einen oder mehrere Farbstoffe umfasst, der Farbstoff vorzugsweise ein organischer Farbstoff ist, ausgewählt aus der Gruppe bestehend aus Akridin-Farbstoffen, AnthrachinonFarbstoffen, Diarylmethan-Farbstoffen, Triarylmethan-Farbstoffen, AzoFarbstoffen, Phtalocyanin-Farbstoffen, Diazo-Farbstoffen, Quinon-Farbstoffen, Azin-Farbstoffen, Indamin-Farbstoffen, Indophenol-Farbstoffen, Oxazin-Farbstoffen, Oxazon-Farbstoffen, Thiazin-Farbstoffen, Thiazol-Farbstoffen, Xanthen-Farbstoffen, Fluoren-Farbstoffen, Rhodamin-Farbstoffen und Fluoron-Farbstoffen und/oder wobei der Farbstoff ein emittierender Farbstoff ist.

13. Kopiergeschütztes Papier nach einem der vorhergehenden Ansprüche, wobei das Papier ausgewählt ist aus der Gruppe, bestehend aus Bankpapier, Zeichenpapier, Druckerpapier, Tintenstrahldruckerpapier, Kopierpapier und Fotopapier.

14. Verfahren zur Herstellung eines kopiergeschützten Papiers nach einem der Ansprüche 1-13, umfassend
- Bereitstellen eines bedruckbaren Papiers, wobei das Papier optional bedruckt ist, sodass das Papier dabei mit einer bedruckten Seite bereitgestellt wird;
- optional Bereitstellen des Papiers mit einer transparenten Schicht auf der zu bedruckenden Seite oder der bedruckten Seite;
a)
- Bereitstellen einer Beschichtungszusammensetzung, optional umfassend ein organisches Polymer, welche Beschichtungszusammensetzung im getrockneten Zustand einen Brechungsindex hat, der sich um mindestens 0,05, vorzugsweise um mindestens 0,1 vom Brechungsindex des bedruckbaren Papiers oder vom Brechungsindex der transparenten Schicht unterscheidet;
- Anwenden der Beschichtungszusammensetzung auf der bedruckten Seite oder einer zu bedruckenden Seite des Papiers; und
- Trocknen der Beschichtungszusammensetzung, um eine transparente Beschichtung bereitzustellen, die 1-50 Gewichtprozent anorganische Partikel mit einer durchschnittlichen Partikelgröße von 0,5-200 nm umfasst, oder
b)
- Anwenden einer transparenten Schicht, die 1-50 Gewichtprozent anorganischer Partikel mit einer durchschnittlichen Partikelgröße von 0,5-200 nm umfasst, auf der bedruckten Seite oder einer zu bedruckenden Seite des Papiers durch einen Gasphasenabscheidungsprozess, wobei die Schicht nach dem Anwenden durch Gasphasenabscheidung einen Brechungsindex hat, der sich um mindestens 0,05, vorzugsweise um mindestens 0,1 vom Brechungsindex des bedruckbaren Papiers oder vom Brechungsindex der optionalen transparenten Schicht unterscheidet.

15. Verwendung einer transparenten Schicht, wie in einem der Ansprüche 1-12 definiert, als Kopierschutz für Informationen, gedruckt auf oder zu drucken auf ein Papier.

## Revendications

1. Papier protégé contre la copie comprenant un papier imprimable présentant, sur une face à imprimer ou une face imprimée, une première couche transparente, dans lequel ladite première couche transparente présente une différence d'indice de réfraction avec
i) ledit papier ; ou avec
ii) une deuxième couche transparente facultative prévue sur ledit papier sur la face à imprimer ou la face imprimée,
dans lequel ladite différence d'indice de réfraction est au moins de 0,05 et
dans lequel la première couche transparente comprend en outre 1 à 50 % en poids de particules inorganiques ayant une taille moyenne de particules comprise entre 0,5 et 200 nm.

2. Papier protégé contre la copie selon la revendication 1, dans lequel la première couche transparente comprend un polymère organique, le polymère organique étant de préférence choisi dans le groupe formé par l'amidon, la cellulose, l'alcool polyvinylique et leurs dérivés.

3. Papier protégé contre la copie selon l'une quelconque des revendications précédentes, dans lequel la première couche transparente comprend en outre des particules inorganiques ayant une taille moyenne de particules comprise entre 0,6 et 100 nm, de préférence entre 0,7 et 50 nm, et dans lequel lesdites particules sont de préférence non sphériques.

4. Papier protégé contre la copie selon la revendication 3, dans lequel lesdites particules non sphériques se présentent sous la forme de plaquettes ayant un rapport largeur/hauteur de 10 ou plus, dans lequel l'orientation des particules est telle que l'angle moyen entre le plan des plaquettes et le plan du papier est inférieur à 60°, de préférence inférieur à 45°, et de préférence encore inférieur à 20°.

5. Papier protégé contre la copie selon l'une quelconque des revendications précédentes, dans lequel ladite différence d'indice de réfraction est au moins de 0,1, de préférence au moins de 0,2, de préférence encore d'au moins 0,5, et de préférence encore comprise entre 0,5 et 1,5.

6. Papier protégé contre la copie selon l'une quelconque des revendications précédentes, dans lequel les particules inorganiques sont sélectionnées dans le groupe formé par TiO₂, SnO₂, Si, Ag, Au, C(diamant), ZnO, ZrO₂, CeO₂, Hf₂O₃, le mica éventuellement revêtu et l'argile éventuellement organiquement modifiée.

7. Papier protégé contre la copie selon l'une quelconque des revendications précédentes, dans lequel la première couche transparente comprend 20 à 40 % en poids, de préférence 30 à 40 % en poids, de particules inorganiques.

8. Papier protégé contre la copie selon l'une quelconque des revendications précédentes, dans lequel l'épaisseur totale de la somme des couches transparentes est au maximum de 1 000 nm, de préférence au maximum de 500 nm, et de préférence encore au maximum de 200 nm.

9. Papier protégé contre la copie selon l'une quelconque des revendications précédentes, comprenant au moins 2 couches transparentes, de préférence 2 à 20 couches transparentes, la couche transparente la plus proche du papier contenant de préférence du mica, de préférence du mica revêtu de dioxyde de titane rutile, d'oxyde d'étain et/ou d'oxyde de fer.

10. Papier protégé contre la copie selon l'une quelconque des revendications précédentes, dans lequel les particules inorganiques ont un indice de réfraction d'au moins 0,4, de préférence d'au moins 1,0, de préférence encore compris entre 1,0 et 4,0, et idéalement compris entre 2,0 et 4,0 tel que mesuré par un réfractomètre.

11. Papier protégé contre la copie selon l'une quelconque des revendications précédentes, dans lequel la surface des particules inorganiques est modifiée par un ou plusieurs composés organiques, ledit un ou plusieurs composés organiques comprenant de préférence des groupes ammonium, phosphonium, carboxyles, siloxane et/ou hydroxyles.

12. Papier protégé contre la copie selon l'une quelconque des revendications précédentes, dans lequel ladite première couche transparente comprend un ou plusieurs colorants, ledit colorant étant un colorant organique choisi dans le groupe formé par les colorants acridiniques, les colorants anthraquinoniques, les colorants diarylméthaniques, les colorants triarylméthaniques, les colorants azoïques, les colorants phtalocyaniniques, les colorants au diazonium, les colorants quinoniques, les colorants aziniques, les colorants indaminiques, les colorants indophénoliques, les colorants oxaziniques, les colorants oxazoniques, les colorants thiaziniques, les colorants thiazoliques, les colorants xanthéniques, les colorants au fluorène, les colorants rhodaminiques et les colorants à la fluorone, et/ou dans lequel ledit colorant est un colorant émetteur.

13. Papier protégé contre la copie selon l'une quelconque des revendications précédentes, dans lequel le papier est choisi dans le groupe formé par le papier de banque, le papier à dessin, le papier d'imprimante, le papier pour jet d'encre, le papier pour photocopieur et le papier photographique.

14. Procédé de préparation d'un papier protégé contre la copie selon l'une quelconque des revendications 1 à 13, consistant à
- fournir un papier imprimable, ledit papier étant à titre facultatif imprimé et donc fournir ledit papier avec une face imprimée ;
- doter à titre facultatif ledit papier d'une couche transparente sur la face à imprimer ou sur la face imprimée ;
a)
- fournir une composition de revêtement, comprenant à titre facultatif un polymère organique, ladite composition de revêtement, une fois sèche, ayant un indice de réfraction qui diffère d'au moins 0,05, de préférence d'au moins 0,1, de l'indice de réfraction dudit papier imprimable ou de l'indice de réfraction de ladite couche transparente ;
- appliquer ladite composition de revêtement sur la face imprimée ou sur une face à imprimer dudit papier ; et
- faire sécher ladite composition de revêtement pour fournir un revêtement transparent comprenant 1 à 50 % en poids de particules inorganiques ayant une taille moyenne de particules comprise entre 0,5 et 200 nm, ou
b)
- appliquer une couche transparente comprenant 1 à 50 % en poids de particules inorganiques ayant une taille moyenne de particules comprise entre 0,5 et 200 nm sur la face imprimée ou sur une face à imprimer dudit papier par un processus de dépôt en phase gazeuse, ladite couche, après avoir été appliquée par dépôt en phase gazeuse, ayant un indice de réfraction qui diffère d'au moins 0,05, de préférence d'au moins 0,1, de l'indice de réfraction dudit papier imprimable ou de l'indice de réfraction de ladite couche transparente facultative.

15. Utilisation d'une couche transparente telle que définie dans l'une quelconque des revendications 1 à 12 comme protection contre la copie des informations imprimées ou à imprimer sur un papier.
